

## UNITED STATES PATENT OFFICE

2,474,785

PROCESS FOR PRINTING WITH SULPHURIC  
ESTERS OF LEUCO VAT DYESTUFFS

William B. Hardy and Elizabeth M. Hardy, Bound Brook, N. J., assignors to American Cyanamid Company, New York, N. Y., a corporation of Maine

No Drawing. Application July 31, 1946,  
Serial No. 687,520

7 Claims. (Cl. 8—70)

1

This invention relates to an improved process for printing textile fibers and fabrics with difficultly oxidizable sulfuric ester salts of leuco vat dyes using the dichromate-acid vapor developing method.

Printing of textiles with sulfuric ester salts of leuco vat dyes has been carried out by two general procedures. One of the processes incorporates a powerful oxidizing agent in the printing paste, such as a chlorate, and the print is developed by treatment with steam and acid vapors. This process is generally usable with all stable dyestuffs. However, it is open to a very serious disadvantage when the dye mixture printed contains dyes which are sensitive to oxidizing agents. In the process such colors are rather severely attacked and the use of processes involving strong oxidizing agents such as chlorates have, therefore, been definitely limited in their field of utility.

Some of the disadvantages of the chlorate acid vapor process are overcome by a procedure in which a milder oxidizing agent, such as a dichromate, is incorporated into the printing paste containing sulfuric esters of leuco vat dyestuffs, and aging effected with acid vapors, such as, for example, mixed acetic acid-formic acid vapors. It is with this dichromate process that the improvement of the present invention deals.

The dichromate-acid vapor process, while it does not attack sensitive dyes, is also subject to a number of drawbacks. The principal one is that certain sulfuric esters of leuco vat dyestuffs which are difficultly oxidizable do not fully develop during the acid vapor treatment within the usual aging periods of about 1-5 minutes, even when large excesses of the oxidizing agent are used. Also, drastic increases in the aging time, e. g., up to 20 minutes, do not bring about full development. A further drawback is that development of the incompletely developed color sometimes continues slowly during after-storage of the fabric which results in a change of shade. As a result of the above drawbacks the dichromate-acid vapor process has been restricted to sulfuric esters of leuco vat dyes which are readily oxidizable, and has been considered unsuitable for a large field of difficultly oxidizable esters, especially those derived from indigos and thioindigos which contain negative substituents. As a result the dichromate-acid vapor process has not been usable with a certain class of sulfuric esters of leuco vat dyes, including some of the important vat colors.

According to the present invention it has been 55

2

found that full development in a short time is obtained by the dichromate-acid vapor process with difficultly oxidizable sulfuric esters of leuco vat dyestuffs when there is added to the paste an alkyl or alkenyl aniline sulfonic acid or a water-soluble salt thereof, which are to be regarded as equivalents. Since it is the substituted aniline sulfonic acid radical which is effective regardless of whether this radical is attached to hydrogen to form the free acid or to a basic radical to form a salt, the term "aniline sulfonic acid radical" will be used in the claims to cover either type of compound, and it will be used therein in no other sense.

15 The substituent in the aniline sulfonic acid is an aliphatic hydrocarbon radical having not more than one double bond. There may be present one substituent or a plurality. The sulfonic acids which may be considered as development 20 accelerators or catalysts may be added either to the printing paste or to the dry ester salts used in preparing a printing formula. When properly used, fast prints are obtained of excellent strength and brilliance, the dyeing strength being increased in many cases from values as low as 10% to substantially the full color value.

Improved results of the present invention are obtained regardless of whether the alkyl or alkenyl group or groups are attached to a carbon atom of the benzene ring or to the nitrogen atom. 30 This is unusual because ordinarily the presence of an alkyl or alkenyl group produces chemical compounds of quite different characteristics, depending on whether it is a ring substituent or is attached to the nitrogen. It is not known why the contrary is the case in the process and compositions of the present invention, and it is not desired to limit the same to any theory. Among the typical compounds included in the present 35 invention are sulfonic acids of toluidines, xyli- 40 dines, cumidines, cymidines and N-mono and dialkyl or alkenyl anilines, such as diethylaniline, diallylaniline, and the like. The position of the sulfonic acid does not appear to be vital. 45 There is some variation in degree of positive results obtained with individual members of the substituted aniline sulfonic acids of the present invention, but the class as a whole gives useful improvements in printing with difficultly oxidizable sulfuric esters of leuco vat dyestuffs. It is an advantage of the present invention that the added compounds do not themselves form disturbing oxidation colors under the conditions of operation.

The improved results which are obtainable

with the printing assistants of the present invention appear to be quite specific to the class. Normally, the chemical behavior of alkyl substituted compounds and aralkyl substituted compounds is quite similar. In the present case this does not hold true and sulfonic acids of N-benzyl anilines do not show the great improvement which is typical of the compounds of the present invention. The underlying chemical reason for this sharp difference is not as yet proven, and no theory is advanced why such closely related aralkyl derivatives do not possess the valuable properties of the assistants of the present invention.

The properties of an oxidation accelerator or catalyst, which are so marked in the substituted aniline sulfonic acids of the present invention, are quite surprising because the same general type of compound has been used in processes of printing with other and stronger oxidizing agents, such as chlorates. In such a process the compounds exert the opposite effect and prevent over-oxidation, particularly when used in a process in which development is effected by steaming and not by acid vapors. The reasons for the contrary effects in the different processes are likewise not known.

It should be emphasized that the process of the present invention is strictly limited to an improved dichromate-acid vapor printing process in which leuco vat dye ester salts are used which are difficultly oxidizable in this process. It should not be confused with processes in which development is effected by passing the printed goods through a liquid bath containing an oxidizing agent, such as nitrite or dichromate. In general, vat dye ester salts which are difficult to oxidize by this bath process are also difficult to oxidize by the dichromate-acid vapor process. There are, however, a few exceptions where a leuco vat dye ester salt is fairly readily oxidized by the bath process and is difficultly oxidizable by the dichromate-acid vapor process, requiring one of our catalysts for full development.

It is an advantage of the present invention that the amount of oxidation accelerator or dyeing assistant is not critical. Apparently, the compound does not take part strictly as a reactant, and a considerably smaller amount of the accelerator may be used than oxidizing agent. In general an amount of accelerator which is somewhat less than the weight of the dyestuff ester gives best results. However, good results are obtained from quite a wide range of proportions. It is, of course, necessary to add sufficient accelerator to produce rapid oxidation, the minimum amount varying with different accelerators and with different dyes. Small traces of accelerator are, of course, not effective, as the reaction appears not to be a purely catalytic one in which minute quantities of accelerator are capable of carrying on the reaction of very large amounts of dyestuff and oxidizer.

It is an advantage of the present invention that the prints are not only of excellent strength and brilliance, the strength being increased in many cases from as low as 10% to substantially full color value, but that the process is controllable, that is to say, the rate of development can be influenced by the addition of varying amounts of accelerator. Thus, prints can be made to develop in a shorter time than normal, for example, in a few minutes, or the color development may be caused to proceed more slowly so that the reaction rate can be controlled within wide limits, in accordance with the desire of the opera-

tor. In every case prints are obtained which show improved levelness and freedom from specks, and they do not show any deterioration in shade due to after development. It is a further advantage of the invention that the accelerator permits operation without a larger excess of oxidizing agent.

The invention will be described in greater detail in conjunction with the following examples, which are typical. The parts are by weight.

#### Example 1

15 7 parts of the sodium salt of the disulfuric acid ester of leuco tetrabromoindigo (equivalent to 4.35 parts of tetrabromoindigo) are blended with 2 parts of 2-amino, 3-5-dimethylbenzene sulfonic acid (Na salt) and 1.1 parts of sucrose to give a powder containing approximately 43% real dye.

20 A printing paste is made from this blended powder, using the following ingredients:

|                                                                                           | Parts |
|-------------------------------------------------------------------------------------------|-------|
| Color                                                                                     | 3     |
| Urea                                                                                      | 6     |
| 25 A mixture of 4 parts acetamide, 4 parts diethylene glycol and 2 parts furfuryl alcohol | 3     |
| Water                                                                                     | 11    |
| A 15% gum paste in water                                                                  | 70    |
| 30 Ammonium chloride                                                                      | .75   |
| 25% ammonia                                                                               | 2.0   |
| Sodium dichromate                                                                         | 5.0   |

35 The cloth is printed with this paste and the resulting prints are aged in formic and acetic acid vapors. The prints develop to substantially full color value, in 1 to 3 minutes. If no metaxylidine sulfonic acid is present in the powder, only 10-15% of the expected color value is obtained even after as long as 10 minutes aging.

#### Example 2

40 7 parts of the crude sodium salt of the disulfuric ester of leuco tetrabromoindigo (equivalent to 4.35 parts of tetrabromoindigo) are blended with 2 parts of sodium 2-amino-5-methylbenzene sulfonate and 1.1 parts of sucrose to give a powder containing approximately 43% real dye. When this powder is incorporated into a printing 45 paste as described in Example 1, printed and aged, prints of substantially full color value were obtained. In the absence of the sodium p-aminotoluene sulfonate only about 10% of the expected color value is obtained.

#### Example 3

55 6 parts of crude sodium salt of the disulfuric ester of leuco tetrabromoindigo (equivalent to 3.59 parts of tetrabromoindigo) were blended with 2 parts of sodium N,N-diethylaniline 4-sulfonate and 0.28 part of sucrose to give a powder of approximately 43% dye content. Prints obtained from this product by the usual 60 procedure of printing and dyeing described in Example 1, develop to full color value on short aging. Only a small fraction (about 10%) of the desired color value can be obtained in the absence of sodium diethylaniline sulfonate.

70 Sodium diethylaniline sulfonate also greatly increases the printing strength of the blended powder of the sodium salt of the disulfuric ester of leuco 7,7'-dimethyl - 5,5' - dichlorothioindigo over that of a similar powder containing no 75 sodium diethylaniline sulfonate.

## Example 4

7 parts of the crude sodium salt of the disulfuric ester of leuco tetrabromoindigo (equivalent to 4.19 parts of tetrabromoindigo) are blended with 2 parts of sodium N,N-diallylaniline sulfonate and 0.66 parts of sucrose, to give a powder of 43% dye content. This product on printing and aging by the procedure described in Example 1, gives prints of essentially full strength on short aging. The required color value is not obtained under identical conditions in the absence of sodium diallylaniline sulfonate.

## Example 5

7 parts of the sodium salt of the disulfuric acid ester of leuco 7,7'-dimethyl-5,5'-dichlorothioindigo (containing 3.9 parts of 7,7'-dimethyl-5,5'-dichlorothioindigo) are blended with 1.66 parts of 2-amino 3,5-dimethylbenzene sulfonic acid sodium salt to give a powder of approximately 44% real dye content. Prints obtained from this powder by the procedure described in Example 1 develop to substantially full color value on 1 to 3 minutes aging. In the absence of the meta-xylidine sulfonic acid sodium salt, only 10 to 20% of the expected color value is obtained after 10 minutes aging.

If the meta-xylidine sulfonic acid sodium salt in the above example is replaced by the sodium salt of N-benzyl sulfanilic acid only about 20% of the expected color value is obtained after 10 minutes aging.

## Example 6

9 parts of the sodium salt of the disulfuric acid ester of leuco 4,5,4',5'-dibenzthioindigo (containing 4.67 parts of real 4,5,4',5'-dibenzthioindigo) are blended with 1.38 parts 2-amino 3,5-dimethylbenzene sulfonic acid sodium salt to give a powder containing approximately 45% real dye. Prints of substantially full color value are obtained from this powder by means of the previously described printing formula and in an aging time of 1 to 3 minutes. If no meta-xylidine sulfonic acid sodium salt is included in the powder, only 10 to 20% of the expected color value is obtained even after a 10 minute aging.

The leuco vat dye ester salt used in this example constitutes one of the few exceptions referred to in the introductory portion of the specification. This ester salt has been characterized in the literature as being fairly readily oxidizable in liquid development processes where the leuco ester salt is used primarily for dyeing rather than printing. In the dichromate-acid vapor process of developing prints this leuco ester salt is to be characterized as difficultly oxidizable since it will not develop to full color value in a reasonable time

without the use of the accelerators of the present invention.

## Example 7

4.7 parts of the sodium salt of the disulfuric ester of leuco 4,4'-dimethyl-6,6'-dichlorothioindigo (containing 2.55 parts of real dye) are blended with 1.05 parts of 2-amino 3,5-dimethylbenzene sulfonic acid sodium salt and 1.54 parts of sucrose to give a powder containing 36% real dye. Prints obtained from this product by the procedure described in Example 1 give essentially the full color value on aging for 1 to 3 minutes. In the absence of the meta-xylidine sulfonic acid, only a 5% to 10% of the expected color value is obtained even after 10 minutes aging.

We claim:

1. A process for printing difficultly oxidizable sulfuric ester salts of leuco vat dyestuffs of the indigoid type which comprises printing the ester salts with dichromates and in the presence of an effective amount of an aniline sulfonic acid radical, substituted by at least one aliphatic hydrocarbon radical containing not more than one double bond, and developing the print with acid vapors.
2. A process according to claim 1 in which the substituted aniline sulfonic acid is 2-amino-3,5-dimethylbenzene sulfonic acid.
3. A process according to claim 1 in which the substituted aniline sulfonic acid is N,N-diethyl-aniline-para-sulfonic acid.
4. A process according to claim 1 in which the substituted aniline sulfonic acid is a para-toluidine sulfonic acid.
5. A process according to claim 1 in which the sulfuric ester salt is the disulfuric ester salt of leuco tetrabromoindigo.
6. A process according to claim 1 in which the sulfuric ester salt is the disulfuric ester salt of a dimethyl-dichlorothioindigo.
7. A process according to claim 1 in which the sulfuric ester salt is the disulfuric ester salt of leuco 4,5,4',5'-dibenzthioindigo.

WILLIAM B. HARDY.  
ELIZABETH M. HARDY.

## REFERENCES CITED

The following references are of record in the file of this patent:

## UNITED STATES PATENTS

| Number    | Name                | Date          |
|-----------|---------------------|---------------|
| 1,779,305 | Brandt _____        | Oct. 21, 1930 |
| 2,234,301 | Niederhausern _____ | Mar. 11, 1941 |

## FOREIGN PATENTS

| Number  | Country      | Date          |
|---------|--------------|---------------|
| 398,571 | France _____ | Mar. 26, 1909 |